

## UNITED STATES PATENT OFFICE.

EUGENE L. MAUPAI, OF NEW YORK, N. Y.

## PROCESS OF DYEING SILK.

No Drawing.

Application filed February 1, 1926. Serial No. 85,380.

This invention relates to an improvement in the dyeing of colors that will be absolutely fast to boiling soap solution and fast to peroxide of hydrogen bleach (such as is commonly used in the textile dyeing plants) also fast to perspiration, on silk piece goods and skein silk, with dyes such as chromogene, autochrome, indigosol or similar dyes that can be employed with the addition of a metallic salt, such as bichromate of potassium, or copper sulphate, in the same bath or in a separate bath after dyeing. The chromogene and autochrome dyes referred to above are monoazo dyes, while the indigosol is an indigoid dye.

Heretofore no successful way has been found of dyeing silk piece goods or skein silk absolutely fast, with such dyes as stated above, and furthermore I have found that silk could not heretofore be successfully dyed with the above named dyes and metallic salts in the same bath as the colors would not come out with any degree of brilliancy. By my improved process as will presently be described, I am able to dye silk any shade absolutely fast to a boiling soap solution.

The process is conducted as follows:

The silk piece goods or skein silk are treated in a bath containing the chromogene or such similar colors, in accordance with the shade desired, with the addition of from 3 to 10% acetic acid or 3 to 5% sulfuric acid, depending upon the color. The dyebath is started cold and gradually raised to a boiling point temperature, whereupon 3 to 5% of a metallic salt such as above, is added. The goods are worked in this manner for about 30 minutes and then gradually brought to a boil within about 40 minutes.

After the dyeing process and the treatment with the metallic salt the skein silk or piece goods are thoroughly rinsed and thereupon entered into a boiling, highly concentrated soap solution at approximately boiling point, by which the color is developed.

The silk may be first dyed in a bath with either a chromogene or autochrome or indigosol dye or such dyes that will stand metallic salt treatment, or in a separate bath of metallic salts, after dyeing with above colors. Then the colors are developed and fixed by the soap boiling process above described.

Summarizing my process I employ the following steps:

- A. Dyeing the silk with either of above dyes or similar ones;
- B. Treating the silk in the same dyebath with a metallic salt, or applying the metallic salt in a separate bath after dyeing.
- C. Rinsing the silk after the metallic salt treatment; and finally
- D. Boiling the silk in a highly concentrated soap solution, which develops and fixes the colors.

Wherever in the claims I refer to any of the dyes mentioned in the specification, I intend that any dye of like character may be substituted as an equivalent.

By my invention I am able to dye silk piece goods or skein silk any shade, the color being absolutely fast to boiling soap solution and peroxide hydrogen bleach, and the process applies to both colors and black.

Having now described my invention, what I claim is:

1. A step in the process of dyeing silk with a dye of the class including chromogene, autochrome, and indigosol, and a metallic salt having oxidizing properties, which comprises redeveloping previously dyed silk in a highly concentrated boiling soap solution.
2. A process of dyeing silk with a dye of the class including chromogene, autochrome, and indigosol, which comprises treating the dyed silk with a metallic salt having oxidizing properties, and finally developing the silk with a highly concentrated soap solution.
3. The process of dyeing silk material with a dye of the class including chromogene, autochrome, and indigosol, which comprises first subjecting the silk to the action of a bath containing a metallic salt having oxidizing properties, then boiling the silk in this bath at the boiling point, then rinsing the silk, and finally developing the color in a highly concentrated boiling soap solution.

4. The process of dyeing silk with a dye of the class including chromogene, autochrome, and indigosol, which comprises treating the silk in the dyebath with a metallic salt having oxidizing properties, and finally boiling the silk in a highly concen-

- trated soap solution to develop and fix the color.
5. The process of dyeing silk with a dye of the class including chromogene, autochrome, and indigosol, which comprises applying a metallic salt having oxidizing properties in a separate bath, after dyeing, rinsing the silk after the metallic salt treatment, and finally boiling the silk in a highly concentrated soap solution to develop and fix the color.
6. Silk dyed with a dye of the class including chromogene, autochrome, and indigosol, and fast to a boiling soap solution and a peroxide hydrogen bleach.
7. Silk dyed with a azo dye of the class including chromogene, autochrome, and indigosol which will be fast to a boiling soap solution.
8. Silk dyed with a dye of the class including chromogene, autochrome and indigosol which will be fast to a peroxide of hydrogen bleach.

EUGENE L. MAUPAI.